

April 16, 1940.

H. DAVIS ET AL

2,197,098

MANDREL

Filed Dec. 7, 1936

FIG.1.



FIG.2.



FIG.3.



FIG.4.



FIG.6.



FIG.5.



Inventors:

HERBERT DAVIS and  
JOSEPH PAWOL.

by: *Usina & Rauher*  
their Attorneys.

## UNITED STATES PATENT OFFICE

2,197,098

## MANDREL

Herbert Davis, Cleveland, Ohio, and Joseph Pawol, Ellwood City, Pa., assignors to National Tube Company, a corporation of New Jersey

Application December 7, 1936, Serial No. 114,714

## 5 Claims. (Cl. 148—3)

- This invention relates to mandrels for metal-working operations and more particularly to piercing points and plugs for use in seamless tube mills.
- 5 In the manufacture of pipes and tubes heretofore, it has been impossible to successfully pierce solid billets made of high-chromium and high-chromium-nickel alloys of the stainless type, with piercing points made of low-chromium-nickel alloys. The conventional chromium-nickel piercing points, upon repeated usage on short length billets; or single usage on long lengths of plain or alloy tubing; or single usage on stainless steel, fail by either distorting, burning on the 15 nose, welding to the billet, picking-up metal or cracking from heat. The change in contour materially affects the quality of billet processed, power required, and may at times stall the machine and result in material damage.
- 20 Further, it has been impossible to use this conventional type of piercing point metal analysis on rotary rolling-mills or Stiefel expanding-mills, wherein a finished wall-size is obtained, due to the necessity and difficulty of machining 25 the plugs to a close tolerance.

The novel mandrel of this invention is especially adaptable for use as a point or plug for piercing all workable plain and alloy steels or metals with a substantial increase in service over 30 the chromium-nickel alloy piercing points heretofore used for both plain and alloy tubing.

The scaling and physical properties of this alloy mandrel, piercing point or plug are, upon heat-treatment, of such character that it is 35 capable of withstanding high thermal shock without deforming, welding, cracking or otherwise becoming useless for more than one operation in a sequence. This has been impossible with the high alloy type of tools heretofore used 40 for piercing alloy steels of the high-chromium and high-chromium-nickel type, as this type of piercing point or plug requires preheating before use to reduce the thermal shock, and was capable of piercing only one piece of material before de- 45 forming, welding or cracking, which renders it unfit for further use.

The physical properties of this alloy when properly heat-treated are exceptionally good, and heat-treated tools formed of this alloy may be 50 shaped, forged, machined, ground or otherwise hot or cold formed without material change of its properties. These properties render the alloy adaptable for rotary rolling mill plugs which must be machined to a close tolerance.

55 Furthermore, with proper heat treatment, this alloy is free from "hot" or "cold shortness" and also from the so-called "blue brittleness" which has long been the bane of points cast from the conventional chromium-nickel alloy irons or 60 steels.

The scaling properties of this alloy mandrel are far superior to the chromium-nickel alloy type. When properly heat-treated, the scale is of a heavy, tightly adherent nature that will not fall off in ordinary handling and, due to a unique 5 property of the scale, when the tool is used it melts or fuses into a hard blue-black lustrous metallic coating which protects the tool during subsequent uses.

The above and further objects will become apparent by referring to the following description and the accompanying drawing, in which:

Figures 1 through 6 are plans of pipe or tube mill piercing points which may be composed of the alloy of the present invention.

15 The piercing point or plug A of Figure 1 is of a type for use with a thirty-six inch roll piercing mill. The point A is composed of an integral casting of the special alloy to be described below and comprises a point portion 2, a tapered body 20 portion 3, and a sleeve or neck portion 4 of less diameter than the body and adapted to receive the forward end of the plug-bar of the mill.

The piercing point or plug B of Figure 2 is another type for use with the thirty-six inch roll 25 piercing mill. The point B is generally of a smaller diameter than the point A and is for piercing smaller billets. The point B consists of a tapered body 5 and a neck or sleeve 6 having a core 7 which is extended into the body portion 30 to receive the end of the plug-bar.

The plug or point C of Figure 3 is for use with a "disk" type of piercing mill and comprises a long tapered nose portion 9 and a body-portion 10 composed of a relatively short straight portion 35 12 and a rearwardly tapered portion 13. The portion 13 is provided with a core 14 to receive the end of the usual plug-bar.

The plug or point D of Figure 4 is for use on a rotary rolling mill or "Stiefel" type cone expander and comprises an angular inlet section 15, a rolling section 16 and a cylindrical section 17. The tool has a cored inlet 18, outlet 19 and chamber 20. The cored section receives the plug 40 supporting mandrel.

The plug or point E of Figure 5 consists of a curvilinear inlet or working section 21, a relief section 22 and core 23 to receive the bar cap.

The plug or point F of Figure 6 consists of a curvilinear inlet or working section 24, a relief 50 section 25 and a chamber core section 26 to receive the bar and reduce the weight.

Plugs or points like the foregoing, or any other design of plug or point, for seamless mill operations, when made in accordance with this invention, are particularly adapted for processing plain or high-chromium or high-chromium-nickel steel alloys of the stainless type or other alloy tubing.

The plugs or points of this invention are cast from an alloy having the following range of analysis:

|                  | Per cent    |
|------------------|-------------|
| 5 Carbon         | .15 to .50  |
| Manganese        | .40 to 1.50 |
| Silicon          | .40 to 1.50 |
| Chromium         | .50 to 2.50 |
| Cobalt           | .50 to 2.50 |
| 10 Copper        | .50 to 2.50 |
| Nickel           | .05 to 2.50 |
| Phosphorus under | .06         |
| Sulphur under    | .06         |
| Iron to make     | 100.00      |

15 Other elements such as aluminum, titanium, zirconium, molybdenum, tungsten or vanadium may be added as desired.

A preferred specific alloy for the plugs or 20 points has the following analysis:

|              | Per cent |
|--------------|----------|
| Carbon       | .20      |
| Manganese    | .75      |
| Silicon      | 1.00     |
| 25 Chromium  | 1.50     |
| Cobalt       | 1.00     |
| Copper       | 1.00     |
| Nickel       | .50      |
| Phosphorus   | .01      |
| 30 Sulphur   | .01      |
| Iron to make | 100.00   |

After the points or plugs are cast from the alloy above set forth, they are heat-treated by 35 annealing in a closed furnace at a temperature between 900 degrees to 1000 degrees centigrade and preferably at approximately 950 degrees centigrade for approximately five hours and slowly cooled in the furnace. This heat treatment materially increases the physical properties 40 of the points or plugs and forms thereon a close adherent scale that becomes a lustrous metallic coating when the tools are used in seamless operations.

45 While we have shown and described several specific embodiments of our invention, it will be understood that we do not wish to be limited exactly thereto, since various modifications may be made without departing from the scope of the invention as defined by the following claims.

50 We claim:

1. The method of making a piercing point for tube mills which includes casting said piercing point from a ferrous alloy having the following 55 analysis:

|                  | Per cent    |
|------------------|-------------|
| Carbon           | .15 to .50  |
| Manganese        | .40 to 1.50 |
| Silicon          | .40 to 1.50 |
| 60 Chromium      | .50 to 2.50 |
| Cobalt           | .50 to 2.50 |
| Copper           | .50 to 2.50 |
| Nickel           | .05 to 2.50 |
| Phosphorus under | .06         |
| 65 Sulphur under | .06         |
| Iron             | Remainder   |

annealing said piercing point at a temperature between 900 degrees and 1000 degrees centigrade and slowly cooling the same, whereby there is 70 formed a tightly adherent scale which melts or fuses when the piercing point is used.

2. The method of making a piercing point for tube mills which includes casting said piercing point from a ferrous alloy having the following 75 analysis:

|                         | Per cent  |
|-------------------------|-----------|
| Carbon approximately    | .20       |
| Manganese approximately | .75       |
| Silicon approximately   | 1.00      |
| Chromium approximately  | 1.50      |
| Cobalt approximately    | 1.00      |
| Copper approximately    | 1.00      |
| Nickel approximately    | .50       |
| Phosphorus under        | .06       |
| Sulphur under           | .06       |
| Iron                    | Remainder |

annealing said piercing point at a temperature between 900 degrees and 1000 degrees centigrade and slowly cooling the same, whereby there is formed a tightly adherent scale which melts or 15 fuses when the piercing point is used.

3. The method of making a piercing point for tube mills which includes casting said piercing point from a ferrous alloy having the following 20 analysis:

|                  | Per cent    |
|------------------|-------------|
| Carbon           | .15 to .50  |
| Manganese        | .40 to 1.50 |
| Silicon          | .40 to 1.50 |
| Chromium         | .50 to 2.50 |
| Cobalt           | .50 to 2.50 |
| Copper           | .50 to 2.50 |
| Nickel           | .05 to 2.50 |
| Phosphorus under | .06         |
| Sulphur under    | .06         |
| Iron             | Remainder   |

annealing said piercing point at a temperature of approximately 950 degrees centigrade and slowly cooling the same, whereby there is formed a tightly adherent scale which melts or fuses 35 when the piercing point is used.

4. The method of making a piercing point for tube mills which includes casting said piercing point from a ferrous alloy having the following analysis:

|                         | Per cent  |
|-------------------------|-----------|
| Carbon approximately    | .20       |
| Manganese approximately | .75       |
| Silicon approximately   | 1.00      |
| Chromium approximately  | 1.50      |
| Cobalt approximately    | 1.00      |
| Copper approximately    | 1.00      |
| Nickel approximately    | .50       |
| Phosphorus under        | .06       |
| Sulphur under           | .06       |
| Iron                    | Remainder |

annealing said piercing point at a temperature of approximately 950 degrees centigrade and slowly cooling the same, whereby there is formed a tightly adherent scale which melts or fuses 55 when the piercing point is used.

5. The method of making a piercing point for tube mills which includes casting said piercing point from a ferrous alloy having the following analysis:

|                  | Per cent    |
|------------------|-------------|
| Carbon           | .15 to .50  |
| Manganese        | .40 to 1.50 |
| Silicon          | .40 to 1.50 |
| Chromium         | .50 to 2.50 |
| Cobalt           | .50 to 2.50 |
| Copper           | .50 to 2.50 |
| Nickel           | .05 to 2.50 |
| Phosphorus under | .06         |
| Sulphur under    | .06         |
| Iron             | Remainder   |

annealing said piercing point, and slowly cooling the same, whereby there is formed a tightly adherent scale which melts or fuses when the 70 piercing point is used.

JOSEPH PAWOL  
HERBERT DAVIS. 75